



US005940110A

# United States Patent [19]

Nakamura et al.

[11] Patent Number: 5,940,110

[45] Date of Patent: \*Aug. 17, 1999

[54] **THERMAL HEAD AND METHOD FOR MANUFACTURING SAME**

[75] Inventors: **Yuji Nakamura; Yoshinori Sato; Yoshiaki Saita**, all of Chiba, Japan

[73] Assignee: **Seiko Instruments Inc.**, Japan

[\*] Notice: This patent issued on a continued prosecution application filed under 37 CFR 1.53(d), and is subject to the twenty year patent term provisions of 35 U.S.C. 154(a)(2).

[21] Appl. No.: **08/669,299**

[22] PCT Filed: **Oct. 25, 1995**

[86] PCT No.: **PCT/JP95/02191**

§ 371 Date: **Jul. 15, 1996**

§ 102(e) Date: **Jul. 15, 1996**

[87] PCT Pub. No.: **WO96/13389**

PCT Pub. Date: **May 9, 1996**

[30] **Foreign Application Priority Data**

Oct. 31, 1994 [JP] Japan ..... 6-267424

[51] **Int. Cl.<sup>6</sup>** ..... **B41J 2/335**

[52] **U.S. Cl.** ..... **347/208; 347/203**

[58] **Field of Search** ..... 347/203, 208

[56] **References Cited**

U.S. PATENT DOCUMENTS

4,096,510 6/1978 Arai et al. ..... 357/28

4,719,477 1/1988 Hess ..... 346/140 R  
5,557,313 9/1996 Nakayama et al. ..... 347/203  
5,590,969 1/1997 Nakayama et al. ..... 347/203

FOREIGN PATENT DOCUMENTS

299735 1/1989 European Pat. Off. ..

OTHER PUBLICATIONS

Patent Abstracts of Japan, vol. 3, No. 40, (E-102) Apr. 6, 1979.

Patent Abstracts of Japan, vol. 13, No. 244 (M-834) [3592] Jun. 7, 1989.

Patent Abstracts of Japan, vol. 14, No. 196 (M-964) [4139] Apr. 20, 1990.

Patent Abstracts of Japan, vol. 7, No. 159, (M-228) [1304] Jul. 13, 1983.

Patent Abstracts of Japan, vol. 6, No. 83 (M-130) May 21, 1982.

Patent Abstracts of Japan, vol. 18, No. 272 (M-1610) May 24, 1994.

*Primary Examiner*—Huan Tran  
*Attorney, Agent, or Firm*—Adams & Wilks

[57] **ABSTRACT**

A thermal head comprises an insulative substrate, a heating-element layer disposed over the insulative substrate, at least one electrode disposed over the heating-element layer for supplying power to the heating-element layer, and a protective film disposed over the heating element layer and the electrode. The electrode has a tapered peripheral edge portion, and the protective film has a Vickers hardness of at least 1200 Kg/mm<sup>2</sup> or more.

**8 Claims, 16 Drawing Sheets**





FIG. 1 (a)



FIG. 1 (b)



FIG. 2 (a)  
enlarged sectional view of heat generating portion



FIG. 2 (b)  
sectional view of peripheral edge of electrode



FIG. 3(a)



FIG. 3(b)



FIG. 3(c)



FIG. 3(d)



FIG. 4(a)



FIG. 4(b)



FIG. 4(c)



FIG. 4(d)



FIG. 5(a)



FIG. 5(b)



FIG. 5(c)



FIG. 5(d)



FIG. 6(a)



FIG. 6(b)



FIG. 6(c)



FIG. 6(d)



FIG. 7(a)



FIG. 7(b)



FIG. 7(c)



FIG. 8(a)



FIG. 8(b)



FIG. 8(c)



FIG. 8(d)



FIG. 9(a)



FIG. 9(b)



FIG. 10 (a)  
(PRIOR ART)



FIG. 10 (b)  
(PRIOR ART)

FIG. 11



FIG. 12



FIG. 13



FIG. 14





FIG. 15



FIG. 16

(PRIOR ART)

| taper angle<br>( deg ) | printing<br>durability | resistance<br>to pulse | resistance<br>to corrosion | resistance<br>to scratch |
|------------------------|------------------------|------------------------|----------------------------|--------------------------|
| 9 0                    | ×                      | △                      | ×                          | ×                        |
| 6 0                    | ×                      | ○                      | △                          | ×                        |
| 3 0                    | △                      | ○                      | ○                          | ○                        |
| 1 5                    | ◎                      | ◎                      | ◎                          | ◎                        |
| 8                      | ◎                      | ◎                      | ◎                          | ◎                        |

FIG. 17

| taper angle<br>( deg ) | Vickers hardness of protective film Hv |         |         |         |
|------------------------|----------------------------------------|---------|---------|---------|
|                        | 9 0 0                                  | 1 2 0 0 | 1 5 0 0 | 1 8 0 0 |
| 9 0                    | ×                                      | ×       | ×       | ×       |
| 6 0                    | △                                      | △       | ×       | ×       |
| 3 0                    | △                                      | ○       | ○       | ○       |
| 1 5                    | △                                      | ◎       | ◎       | ◎       |
| 8                      | △                                      | ◎       | ◎       | ◎       |

FIG. 18

## THERMAL HEAD AND METHOD FOR MANUFACTURING SAME

### TECHNICAL FIELD

The present invention relates to a thermal head which is used in heat sensitive recording of facsimile, printer or the like and a method for manufacturing the same.

### BACKGROUND TECHNIQUES

Conventionally, as illustrated in FIGS. 10(a) and 10(b), a glaze layer 2 is provided as a heat accumulation layer on an insulative substrate 1 such as that made of ceramic material. Then, film formations are performed by sputtering or deposition from a heat generating resistor material such as that of Ta system, silicide system, Ni—Cr system or the like and an electrode material such as that of Al, Cr—Cu or Au, whereupon a heat generating resistor 3 and wiring electrodes 12 composed of a common electrode and individual electrodes are formed through performance of patterning in the photolithographing step. Thereafter, in order to prevent oxidation of and provide wear resistance with respect to the heat generating resistor 3, a protective film 9 such as that made of  $\text{SiO}_2$ ,  $\text{Ta}_2\text{O}_5$ , SiAlON,  $\text{Si}_3\text{N}_4$  or SiC is formed by sputtering, ion plating or CVD (Chemical Vapor Deposition) to thereby manufacture a thermal head.

However, in the conventional method for manufacturing a thermal head, since the sectional configuration of a peripheral edge portion of each of the wiring electrodes 12 composed of a common electrode and individual electrodes is almost orthogonal, similar difference in level occurs also in the surface of the protective film 9. In addition, due to a difference in growth process between a protective film for the heat generating resistor 3 and that for the wiring electrode 12 when this protective film is formed, a fault 10 at which the film continuity as viewed in the plane direction is discontinued occurs in the protective film layer.

For this reason, the thermal head that had been manufactured by the above-mentioned manufacturing method had its resistance value increased early in its use, with the result that when printing was performed using this thermal head, such increase in resistance value became a cause of dotting failures, which resulted in that the printing run service life of the thermal head became shorter. Also, it is considered that during printing run, ions in the thermosensitive paper, moisture,  $\text{Na}^+$  ion and  $\text{Cl}^-$  ion in the atmosphere, and the like enter into the thermal head due to the faults 10 of the protective film thereof, with the result that there was the problem that the heat generating resistor 3 and wiring electrodes 12 were corroded and as a result the thermal head had inferior corrosion resistance.

As conventional examples of solving the above-mentioned problems, a manufacturing method wherein a forward end portion of each wiring electrode 12 connected to a heat generating resistor 3 is tapered to thereby decrease the fault and level difference of the protective film (e.g., Published Unexamined Japanese Patent Application No. S-56-129184), a manufacturing method wherein a photo-step and etching step are performed twice or so with respect to a forward end portion of each wiring electrode 12 connected to a heat generating resistor 3 to thereby form this forward end portion into a two-stepped configuration and thereby decrease the level difference of the protective film (e.g., Published Examined Japanese Patent Application No. S-55-30468), a manufacturing method wherein high frequency bias sputtering is added during formation of the protective film to thereby prevent generation of cracks (e.g.,

Published Unexamined Japanese Patent Application No. S-63-135261), etc. have been made publicly known.

However, while in the conventional thermal head a wiring electrode thereof was such that a specific configuration was imparted to only a forward end portion thereof that is connected to the heat generating resistor, the effect thereof upon enhancement of the printing durability and reliability was not sufficient. Namely, faults and level differences in the protective film that result from the level differences in the wiring electrode occur not only in the portion thereof that corresponds to the forward end portion of the wiring electrode connected to the heat generating resistor but also in the portion thereof that corresponds to an entire peripheral edge portion of the wiring electrode in at least a protective-film region.

On the other hand, if the above-mentioned level differences exist, the protective film 9 is likely to be partly broken off or exfoliated from faults 10 thereof due to mechanical stress that is applied to the level difference portion thereof by sliding movement of the thermosensitive paper and pressing force of a platen roller or due to thermal stress that results from a difference in thermal coefficient of expansion between the heat generating resistor portion and the electrode portion. Accordingly, the effect of the sliding movement of the thermosensitive paper and pressing force of the platen roller is exerted not only upon the heat generating resistor but also upon the surrounding areas thereof, with the result that the protective film is likely to be broken off or exfoliated also by way of the peripheral edge portion of the wiring electrode other than the forward end portion thereof. Also, even when scratches have been made by foreign substances having attached to the thermosensitive paper or the like, these foreign substances are caught by the level difference portion of the wiring electrode, with the result that, similarly, exfoliation or the like of the protective film is likely to occur also from a portion of the electrode other than the forward end thereof.

As mentioned above, the protective film was broken off or exfoliated not only from the forward end portion of the electrode but also from the peripheral edge thereof, whereby the printing run service life of the thermal head was caused to become shorter.

Also, while material having high hardness has on one hand been recently used as material of the protective film in order to improve the wear resistance thereof, emphasis has on the other hand been placed on the above-mentioned problems. Particularly, when cladding is applied using a hard protective film, the thermal head cannot receive an external force with high flexibility and it is also difficult to ease the stress. Accordingly, there was the problem that the phenomenon such as exfoliation or the like of the protective film was likely to become prominent.

Conversely, when the hardness of the protective film is low, the wear resistance becomes inferior, with the result that the heat generating resistor is damaged due to wear of the protective film and therefore the printing run service life can no longer be expected to be improved.

Also, there is the likelihood that during printing run, ions in the thermosensitive paper, moisture,  $\text{Na}^+$  ion and  $\text{Cl}^-$  ion in the atmosphere, and the like may enter into the thermal head due to the level difference of the peripheral edge of the electrode. As a result, there was the problem that this entry corroded the heat generating resistor and electrode, with the result that the thermal head became inferior in terms of the corrosion resistance particularly during standby for printing.

Accordingly, an object of the present invention is to provide a thermal head which is arranged such that, in order

to solve the above-mentioned conventional problems, the peripheral edge portion of the electrode thereof is tapered and the level difference on the surface of the protective film is thereby lessened to thereby have no fault therein while having wear resistance, on the other hand.

#### DISCLOSURE OF THE INVENTION

The present invention is directed to providing a thermal head having on an insulative substrate at least a heat generating resistor, wiring electrodes for supplying power to the heat generating resistor and a protective film for clothing the heat generating resistor and the wiring electrodes in ambient areas thereof, wherein the sectional configuration of the wiring electrodes that are in at least a protective-film region near the heat generating resistor is tapered to thereby make less sharp a difference in level of the wiring electrodes with respect to the surface of the substrate and the hardness HV of the protective film to be clad is made to be 1200 Kg/mm<sup>2</sup> (HV 1200) or more in terms of the Vickers hardness.

In the above-constructed thermal head, since the difference in level between the surface of the insulative substrate and the peripheral edge portion of each wiring electrode is gently tapered, the clothability of the protective film is increased with the result that the faults which were likely to occur at the peripheral edge portion of each wiring electrode cease to exist, whereby the protective film comes to have continuity in the plane direction. Further, even when the hardness of the protective film is made as high as Hv 1200 or more in terms of the Vickers hardness, troubles that occur due to exfoliation of the protective film that is made from faults therein which were conventionally likely to occur at the peripheral edge portion of the wiring electrode can be suppressed. Nor does there occur entry of corroding ions or the like into the protective film from the fault portion thereof. As a result, the printing run durability is not only improved but is the environmental reliability also improved simultaneously.

#### BRIED DESCRIPTION OF THE DRAWINGS

FIGS. 1(a) and 1(b) are an enlarged sectional view illustrating a heat generating portion of a thermal head according to the present invention and a sectional view illustrating peripheral edge portions of electrodes thereof respectively;

FIGS. 2(a) and 2(b) are an enlarged sectional view illustrating a heat generating portion of a thermal head according to the present invention and a sectional view illustrating peripheral edge portions of electrodes thereof respectively;

FIGS. 3(a) to 3(d) are explanatory views illustrating manufacturing process steps for manufacturing the thermal head according to the present invention;

FIGS. 4(a) to 4(d) are explanatory views illustrating manufacturing process steps for manufacturing the thermal head according to the present invention;

FIGS. 5(a) to 5(d) are explanatory views illustrating manufacturing process steps for manufacturing the thermal head according to the present invention;

FIGS. 6(a) to 6(d) are explanatory views illustrating manufacturing process steps for manufacturing the thermal head according to the present invention;

FIGS. 7(a) to 7(c) are explanatory views illustrating manufacturing process steps for manufacturing the thermal head according to the present invention;

FIGS. 8(a) to 8(d) are explanatory views illustrating manufacturing process steps for manufacturing the thermal head according to the present invention;

FIGS. 9(a) and 9(b) are explanatory views illustrating manufacturing process steps for manufacturing the thermal head according to the present invention;

FIGS. 10(a) and 10(b) are an enlarged sectional view illustrating a heat generating portion of a conventional thermal head and a sectional view illustrating peripheral edge portions of electrodes thereof respectively;

FIG. 11 is a graphic diagram showing results of printing run test on the thermal head according to the present invention;

FIG. 12 is a graphic diagram showing results of continuous pulse application test on the thermal head according to the present invention;

FIG. 13 is a graphic diagram showing results of electrolytic corrosion test on the thermal head according to the present invention;

FIG. 14 is a graphic diagram showing results of printing thickness test on the thermal head according to the present invention;

FIG. 15 is a view illustrating a contact portion between the thermal head according to the present invention and a recording medium;

FIG. 16 is a view illustrating a contact portion between the conventional head and a recording medium;

FIG. 17 is a table showing results of evaluation made in the embodiment of the present invention; and

FIG. 18 is a table showing results of evaluation concerning a scratch test performed according to the present invention.

#### BEST MODE FOR CARRYING OUT THE INVENTION

##### [First Embodiment]

FIG. 1(a) is an enlarged sectional view illustrating a heat generating resistor and its ambient area of a thermal head according to the present invention and FIG. 1(b) is a sectional view illustrating peripheral edge portions of electrodes thereof.

In these figures, a glaze 2 is formed on the surface of an insulative substrate 1 and wiring electrodes 4 are formed thereon so as to be electrically connected to a heating-element layer such as a heat generating resistor 3. A reference numeral 5 denotes a taper portion of each wiring electrode 4. This taper portion is formed with respect to a periphery thereof that opposes the heat generating resistor 3 and with respect to a peripheral edge portion of every wiring electrodes 4. A reference numeral 9 denotes a protective film which is formed so as to clothe the heat generating resistor 3 and the peripheral edge portions of the wiring electrodes 4. By the section of the peripheral edge of the wiring electrode 4 being tapered, when the protective film 9 has been formed, the protective film is made to have no level difference resulting from the level difference of the wiring electrode 4 and have, by the resulting removal of the difference between the growth process thereof on the heat generating resistor 3 and the growth process thereof on the wiring electrodes 4, no fault resulting therefrom.

Also, in the sectional views of FIGS. 2(a) and 2(b), a glaze 2 is formed on the surface of the insulative substrate 1. On the surface of this glaze 2 there is further formed the heat generating resistor 3 on which the wiring electrodes 4

are formed so as to be electrically connected thereto. A reference numeral 6 denotes a multistage portion which is formed with respect to a periphery thereof that opposes the heat generating resistor 3 and with respect to a peripheral edge portion of every wiring electrode 4.

The reference numeral 9 denotes the protective film which is formed so as to cover this multistage portion as a whole.

By the peripheral edge portion of the wiring electrode 4 being formed into a multistage configuration, when the protective film 9 has been formed, the protective film is made to have no level difference resulting from the level difference of the wiring electrode 4 and have, by the resulting removal of the difference between the growth process thereof on the heat generating resistor 3 and the growth process thereof on the wiring electrodes 4, no fault resulting therefrom.

Explaining the manufacturing process steps according to the invention of this application sequentially, as illustrated in FIG. 3(a), for the purpose of heat accumulation, the glaze 2 is formed on the insulative substrate 1 that consists of, for example, alumina ceramics. Next, a film that is made of material Ta—N, Ta—SiO<sub>2</sub> or the like that has Ta as a main component and that serves as material of the heat generating resistor is formed by sputtering to a thickness of approximately 0.1 μm or so, after which the heat generating resistor 3 is formed by photolithography. Subsequently, a film that is made of material Al, Al—Si, Al—Si—Cu or the like that has Al as a main component and that serves as material of the electrode for supplying power to the heat generating resistor 3 is formed by sputtering or the like to a thickness of approximately 1 to 2 μm or so, after which a photo-resist is coated on the resulting film and then is exposure developed using a photo-mask to thereby form a resist 8 that has a configuration of wiring electrode.

Next, in FIG. 3(b), in an etching solution prepared by adjusting the viscosity of an acidic water mixed solution composed of phosphoric acid, acetic acid, nitric acid, pure water, etc. by adjusting the mixing ratio thereof, when etching the Al film with an etching solution having a low viscosity, this etching solution not only performs Al etching but also is simultaneously carried into an interface between the resist 8 and Al, whereby etching proceeds also in the plane direction of the conductor layer. When the relationship between the etching rate in this plane direction and that in the thicknesswise direction is made to be appropriate, at the time of completion of the etching it is possible to make the peripheral edge portion of the electrode have the taper portion 5.

Thereafter, in FIG. 3(c), the resist 8 is removed using an exfoliation solution such as organic solvent to thereby form the wiring electrodes and taper portion 5.

Next, as illustrated in FIG. 3(d), in order to prevent oxidation of and provide wear resistance to the heat generating resistor 3 and wiring electrodes 4, a film that is made of, for example, a mixture of Si<sub>3</sub>N<sub>4</sub> and SiO<sub>2</sub> is clad by sputtering or the like to a thickness of approximately 3 to 6 μm or so to thereby form the protective film 9.

In the thermal head that is obtained through performance of the above-mentioned process steps, since the peripheral edge portion of the wiring electrode is prevented from being formed into a configuration of cliff and is formed into an appropriately tapered slant surface, it is unlikely that faults occur in the portion of the protective film clothing this taper surface 5 of the wiring electrode that corresponds to the peripheral edge thereof.

Particularly, since sputtering has an inferior characteristic of clothing a level difference, a prominent difference in

terms of the clothability of the protective film occurs between the thermal head of the present invention and the conventional thermal head, whose protective films are both formed by sputtering. This effect will be described later 5 jointly with the results of evaluation.

#### [Second Embodiment]

Next, an explanation will be given of the manufacturing process steps wherein the peripheral edge portion of the wiring electrode is tapered with materials thereof each having Al as a main component being made multilayer as 10 illustrated in FIGS. 4(a) to 4(d).

In FIG. 4(a), as in the case of the first embodiment, the glaze 2 is formed on the insulative substrate 1 such as that made of alumina ceramics or the like and on this glaze 2 there is formed the heat generating resistor 3. Subsequently, an Al electrode 4b film that has Al as a main component and that serves as an electrode material for supplying power to the heat generating resistor 3 is formed as a first layer by sputtering to a thickness of approximately 0.3 to 0.8 μm or 15 so and then an Al alloy electrode 4c film which has Al as a main component and has Si, Cu, Ti and the like added thereto is formed as a second layer by sputtering to a thickness of approximately 0.3 to 0.6 μm or so to thereby form an electrode film having a total thickness of approximately 1 to 2 μm. Thereafter, the resist 8 is formed as in the 20 case of the first embodiment.

Next, in FIG. 4(b), when etching is performed of the first and second layers by use of an etching solution that consists of an acidic water mixed solution composed of phosphoric acid, acetic acid, nitric acid, pure water, etc., since as 25 compared to the Al electrode 4b film as the first layer having Al as a main component the Al alloy electrode 4c film as the second layer wherein Si, Cu, Ti and the like has been added to Al has its crystal grain size made to be very small, the etching rate for this second layer becomes faster. For this reason, etching as viewed in both the plane and thickness directions proceeds, whereby at the etch completion time the peripheral edge portion of the electrode exhibits a tapered 30 configuration. Thereafter, in FIG. 4(c), the resist 8 is removed using an exfoliation solution such as organic solvent to thereby form the wiring electrode and taper portion 5. Thereafter, as in the case of the above-mentioned embodiment, in FIG. 4(d), the protective film 9 is formed. 35

#### [Third Embodiment]

Next, the process steps wherein the crystal grain size of the electrode is caused to vary in the thicknesswise direction and the electrode is thereby tapered as illustrated in FIGS. 5(a) to 5(d) will be explained. In FIG. 5(a), as in the case of the first embodiment, the glaze 2 is formed on the insulative substrate 1 such as that made of alumina ceramics or the like and on the upper surface of this glaze 2 there is formed the heat generating resistor 3. On the upper surface of the resulting structure there is further formed by sputtering to a thickness of from 1 to 2 μm a film that has Al as a main component and that serves as an electrode material for supplying power to the heat generating resistor 3. At this time, the crystal grain size of Al varies due to sputter DC power, substrate temperature, sputter pressure, etc. The 40 crystal grain size of an ordinary Al sputter film is in a range of from 2 to 4 μm. In this embodiment, by controlling the sputter DC power and substrate temperature, the crystal grain size thereof was varied to thereby form an Al electrode 4d film whose crystal grain size varied. In an initial period 45 of the film formation, film formation was performed under ordinary conditions and, as the time lapsed, film formation was performed while the sputter DC power was being

gradually decreased. Since the film forming rate was decreased by the sputter power being decreased, the substrate temperature was decreased. At this time, the crystal grain size in the vicinity of the upper surface of Al was  $0.5 \mu\text{m}$  whereas that in the vicinity of the lower surface thereof was approximately  $2 \mu\text{m}$  or so. Then, on the upper surface of the resulting structure there was formed the resist **8**.

Next, in FIG. 5(b), when Al is etched using an etching solution that consists of, for example, a mixed solution of phosphoric acid, acetic acid, nitric acid and pure water, the etching rate varies due to the variations in crystal grain size in the thicknesswise direction of the film. Namely, the smaller the crystal grain size, the faster the etching rate. For this reason, since etching is performed in both the plane and thickness directions, the peripheral edge portion of the electrode exhibits a configuration of taper at the etch completion time. Thereafter, in FIG. 5(c), the resist **8** is removed using an exfoliation solution such as organic solvent to thereby form the wiring electrode and taper portion **5**. Thereafter, as in the case of the above-mentioned embodiment, in FIG. 5(d), the protective film **9** is formed.

#### [Fourth Embodiment]

Next, the manufacturing process steps wherein the resist forming and etching steps are each performed a plurality of times as illustrated in FIGS. 6(a) to 6(d) to thereby make the peripheral edge portion of the wiring electrode multistage, thereby obtaining an effect similar to that attainable with tapering of the electrode will be explained.

In FIG. 6(a), as in the case of the first embodiment, the glaze **2** is formed on the insulative substrate **1** such as that made of alumina ceramics or the like and on the upper surface of this glaze **2** there is formed the heat generating resistor **3**. On the upper surface of the resulting structure there is further formed by sputtering to a thickness of from 1 to  $2 \mu\text{m}$  a film that has Al as a main component and that serves as an electrode material for supplying power to the heat generating resistor **3**. Thereafter, after formation of a resist **8-1**, in FIG. 6(b), ordinary etching is performed using an etching solution that consists of, for example, an acidic water mixed solution of phosphoric acid, acetic acid, nitric acid, pure water, etc. Further, in FIG. 6(c), the resist **8-1** is removed using an exfoliation solution such as organic solvent to thereby form the wiring electrode **4a**. This wiring electrode **4a** thus formed is a first stage. Next, in FIG. 6(d), a photo-resist is coated again so as to form a second stage of the wiring electrode **4a**, after which the photo-resist is exposure developed using a photo-mask whose exposure pattern contour has been reduced  $5 \mu\text{m}$  or more compared to the contour of the wiring electrode **4a** that has been formed as the first stage of the wiring electrode **4a**, to thereby form a resist **8-2** whose configuration corresponds to that of the wiring electrode as the second stage. Next, in FIG. 7(a), etching is performed using an etching solution that consists of, for example, an acidic water mixed solution of phosphoric acid, acetic acid, nitric acid, pure water, etc. At this time, by completing the etching in 10 to 90% of the thickness of the film, it is possible to impart a step **6** with respect to the wiring electrode **4a**. Thereafter, in FIG. 7(b), the resist **8-2** is removed using an exfoliation solution such as organic solvent to thereby form the two staged wiring electrode **4a**. It is also possible to form a three or more staged wiring electrode **4a** by repeated performance of the above-mentioned steps. Lastly, the protective film **9** is formed. The structure illustrated in FIG. 7(c) is one that has been obtained by forming the protective film **9** on the wiring electrode **4a** that has been obtained in this embodiment. The fact that the level difference of the protective film **9** has been

made smaller than in the prior art has been confirmed. It is to be noted that it is confirmed that the level difference of the protective film is smaller when the level difference of the wiring electrode **4a** is three staged than when this level difference is two staged. That is, by the wiring electrode **4a** being two or three staged, the same effect as that attainable with tapering of the electrode is obtained.

#### [Fifth Embodiment]

Next, the manufacturing process steps wherein the photo-resist developing and etching steps are each performed a plurality of times as illustrated in FIGS. 8(a) to 8(d) to thereby make the peripheral edge portion of the wiring electrode multistage, thereby obtaining an effect similar to that attainable with tapering of the peripheral configuration of the wiring electrode will be explained.

In FIG. 8(a), as in the case of the first embodiment, the glaze **2** is formed on the insulative substrate **1** such as that made of alumina ceramics or the like and on the resulting structure there is formed the heat generating resistor **3**. On the resulting structure there is formed by sputtering to a thickness of from 1 to  $2 \mu\text{m}$  a film that has Al as a main component and that serves as an electrode material for supplying power to the heat generating resistor **3**. Thereafter, a resist **8** is formed, and then, in FIG. 8(b), etching is performed 10 to 90% with respect to the film thickness by using an etching solution that consists of, for example, an acidic water mixed solution of phosphoric acid, acetic acid, nitric acid, pure water, etc. and is finished as is.

Further, thereafter, in the conventional process, the resist **8** is removed using an exfoliation solution such as organic solvent to thereby form the wiring electrode **4a**. However, in this embodiment, since a developing solution has a feature of causing a reduction in amount of the resist **8**, ordinary etching is first performed and then the resulting structure is immersed again in the developing solution to thereby perform second-time development for causing a forced reduction in amount thereof and thereby retreat the resist **8** by a distance of  $5 \mu\text{m}$  or more as illustrated in FIG. 8(c). Next, in FIG. 8(d), etching is performed using an etching solution that consists of, for example, an acidic water mixed solution of phosphoric acid, acetic acid, nitric acid, pure water, etc. and this etching is finished to thereby form a multistage portion **6** with respect to the wiring electrode. Thereafter, in FIG. 9(a), the resist **8** is removed using an exfoliation solution such as organic solvent to thereby form the two staged wiring electrode **4a**.

Further, by repeated performance of the above-mentioned steps it is also possible to form a three or more staged wiring electrode **4a**. Lastly, the protective film **9** is formed.

The structure illustrated in FIG. 9(b) is one that has been obtained by forming the protective film **9** on the wiring electrode **4a** having been obtained in this embodiment. By the extent to which the level difference of the peripheral edge portion of the wiring electrode has changed into a stepped configuration of level difference, the level difference of the protective film is made to be less sharp and in addition the fault thereof that corresponds to the peripheral edge of the wiring electrode is also suppressed. It is to be noted that the level difference of the wiring electrode **4a** in each stage is smaller when this wiring electrode **4a** is three staged than when it is two staged and that, accordingly, the clothability of the protective film is enhanced more in the former case than in the latter. According to the experiments performed by the present inventors, when forming the protective film by an ordinary sputtering method, the clothability of the protective film over the level difference portion, i.e., whether or

not there occurs the fault of the protective film at the level difference portion, remarkably changed depending on whether or not the level difference constituting one stage was to an extent of 0.2 to 0.3  $\mu\text{m}$ . Accordingly, it is preferable that each level difference be suppressed to a value of 0.3  $\mu\text{m}$  or less.

[Evaluations On Each Embodiment]

The results of evaluation on each of the above-mentioned embodiments will hereafter be explained with reference to the tables in FIGS. 17 and 18 which show quality levels of characteristics (e.g., printing durability, resistance to scratch, etc.) of the thermal head at various taper angles 7 shown in FIG. 1. Legends "x", " $\Delta$ ", " $\circ$ " and " $\odot$ " in the tables of FIGS. 17 and 18 represent the quality levels in descending order, with "x" representing a low quality level and " $\odot$ " representing a high quality level.

In a table in FIG. 17, there are shown the results of evaluation on the present embodiments when the taper angle 7 in FIG. 1 has been varied.

In the table in FIG. 17, the "resistance to pulse" is an item of evaluation that is obtained by applying a voltage pulse to the heat generating resistor and determining the degree of change in the resistance value thereof with respect to the number of the pulses applied. The "resistance to corrosion" is an item of evaluation that is obtained by causing the thermal head to contact with a thermosensible paper or chemicals at high temperature and under high humidity and determining whether or not the electrodes are corroded and whether or not the protective film is exfoliated. The "resistance to scratch" is an item of evaluation that is obtained by scratching by use of, for example, sand paper the protective film that includes a portion thereof that is located on the wiring electrodes in the vicinity of the heat generating resistor and thereby evaluating the exfoliation of this protective film. The "printing durability" was evaluated in the percentage of troubles that occurred when continuous printing was performed using a highly wearable poor thermosensible paper containing a large amount of corroding impurities.

From the table in FIG. 17, it can be confirmed that when the taper angle 7 is lower than a border of from 60 to 30 deg., each of the characteristics is rapidly improved. While in the thermal head during a printing run thereof in particular high stresses are produced in the heat generating portion and the peripheral edge portion of the wiring electrode in the vicinity of the heat generating resistor due to heat generated from the heat generating resistor, pressure of the platen roller, sliding movement of the thermosensible paper, etc., as apparent from the table in FIG. 17 the synthetic printing durability that involves therein adverse effects resulting therefrom exhibits a very excellent level when the taper angle is 15 deg. or lower.

While each of the above-mentioned items of evaluation is one that has been obtained when the hardness of the protective film is approximately Hv 1500, the present inventors made their scratch evaluation also on specimens wherein the hardness of the protective film was approximately Hv 900, approximately Hv 1200 and approximately Hv 1800, the results being shown in a table in FIG. 18.

From these results it is understood that in the case of a wiring electrode such as the conventional one whose level difference or taper angle is large and sharp, when it involves scratches, the printing durability does not become very high even when the hardness of the protective film is made to be high. It can be explained that the reason for this is that since the wiring electrode is made of soft material such as Al, the

harder the protective film is, when an external force is locally applied thereto by means of a foreign substance or the like the more in the plane direction of the film this force is transmitted with the result that stresses are concentrated more on the fault portion thereof at the peripheral edge of the wiring electrode. Accordingly, the effect of the present invention is especially prominent on a thermal head wherein the hardness of the protective film is Hv 1200 or more. Regarding the resistance to wear, the protective film whose hardness is high is advantageous and, given that the protective film has continuity as viewed in the plane direction, the resistance to scratch also becomes increased as a result. That is to say, when combined with the hardness of the protective film of Hv 1200 or more, the present invention can exhibit the greatest effect.

The results of evaluation on the above-mentioned embodiments that have been obtained when the taper angle 7 is 15 deg. will now be described in detail.

FIG. 11 shows the results of a printing run duration test 20 that has been performed in the present invention.

In the conventional thermal heads, when the printing run distance has increased up to approximately 50 km or so, exfoliation, chipping-off or the like of the protective film occurs, due to mechanical stress or scratch, from the fault portion thereof that is attributable to the level difference 25 portion of the electrode. As a result, at a point in time when the printing run distance is 100 km, unqualified dots occupied 10% whereas, in the present embodiments, even after a 30 printing run over a distance of 100 km or more, no phenomena such as exfoliation, chipping-off or the like occurred in the protective film. Also, by setting the hardness of the protective film to be Hv 1200 or more, it is possible to suppress the amount of the protective film worn to 2  $\mu\text{m}$  or less. That is, in the present embodiments, various 35 destructions such as exfoliation, chipping-off, wear and the like of the protective film that were conventionally the causes of damaging the thermal heads can be suppressed by tapering of the electrode and increasing in hardness of the protective film, whereby it can be confirmed that the printing durability 40 becomes four times or more as high as that in the prior art, with the result that the printing run performance is improved.

In FIG. 12, there are shown the results of continuous pulse 45 application test in order to evaluate the resistance to pulse of the present invention.

In the conventional thermal heads, the increase in the resistance value becomes 5% or so at a pulses number of 1 $\times$ 108 and becomes 15% or more at a pulses number of 50 6 $\times$ 108. However, in the present embodiments, neither increase nor change in the resistance value is exhibited at even a pulses number of 1 $\times$ 108 and, at even a pulses number of 6 $\times$ 108, the increase in the resistance value is 3% or so, that is, the resistance to pulse is improved. Namely, while conventionally the heat generating resistor became deteriorated due to oxidation or the like by way of the fault portion 55 of the protective film that is attributable to the level difference portion of the electrode, in the present embodiments deterioration of the heat generating resistor has become able to be prevented by tapering of the electrode, whereby it 60 could be confirmed that the resistance to pulse was improved.

FIG. 13 shows the results of electrolytic etching test in 65 order to evaluate the resistance to corrosion of the present invention.

The test was performed as a "leaving-to-stand test" under the conditions that the temperature was 85° C., the humidity

was 85%, the head voltage was 5 V and the thermosensible paper was kept applied. In the conventional thermal heads, unqualified dots generated were large in amount at an early point in time, were 5% or more in 48 hrs and, after lapse of 96 hrs, were approximately 15% whereas in the present embodiments no unqualified dots were admitted in 48 hrs and, even after lapse of 96 hrs, approximately 3% of unqualified dots were only admitted. Namely, in the present embodiments, it could be confirmed that by tapering of the electrode, moisture, ions of the thermosensible paper, etc. were prevented from easy entry into the thermal head, whereby corrosion of the electrode and the like could be prevented with the result that the resistance to corrosion was improved.

Also, compared to the sectional structure of the conventional thermal head as illustrated in FIG. 16, more excellent contact between the protective film on the resistor and a recording medium such as a thermosensible paper, platen roller and the like is obtained by tapering the electrode as in the thermal head of the present invention as illustrated in FIG. 15. In FIG. 14 there are shown the results of a print thickness test that has been performed in the present invention.

From the test results it was confirmed that in the present embodiments approximately 20% or more of reduction in the power used was possible even when obtaining the same recorded print thickness as in the prior art, with the result that the efficiency with which the printing heat was generated was improved.

#### Industrial Utilizability

As explained above, according to the present invention, by the electrode of the thermal head in a region of the protective film thereof having been formed into a tapered configuration, the level difference of this protective film is made to be smaller or less sharp, whereby occurrence of faults therein is suppressed and, particularly by the tapering being combined with the hardness of the protective film that is Hv 1200 or more in terms of the Vickers hardness, the wear resistance is of course improved and further the scratch resistance is also remarkably improved. As a result, the present invention has the advantage of making the printing durability very high and further of also improving the environmental reliability.

Also, the manufacturing method of the present invention that is intended to cause tapering of the sectional configuration of the peripheral edge portion of the wiring electrodes is possible to execute with even no use of a special device such as a bias sputter device. Particularly, if an etching process or other processes wherein necessary features can be imparted to the structure of the electrode are used, the section of the peripheral edge of the electrode can be tapered without causing an increase in the number of the steps.

What is claimed is:

1. A thermal head having on an insulative substrate at least a heat generating resistor, wiring electrodes for supplying power to the heat generating resistor and a protective film disposed over the heat generating resistor and the wiring electrodes in ambient areas thereof; wherein at least a peripheral edge portion of each of the wiring electrodes that is in at least a protective-film region near the heat generating resistor has a taper angle of 15 degrees or less; and wherein the protective film has a Vickers hardness of 1200 Kg/mm<sup>2</sup> or more.

2. A thermal head as set forth in claim 1; wherein the entire peripheral edge of each of the wiring electrodes is tapered and has a taper angle of 15° or less.

3. A thermal head comprising: an insulative substrate; a heating-element layer disposed over the insulative substrate; at least one electrode disposed over the heating-element layer for supplying power to the heating-element layer, the at least one electrode having a tapered peripheral edge portion having a taper angle of 15 degrees or less; and a protective film disposed over the heating-element layer and the at least one electrode, the protective film having a Vickers hardness of at least 1200 Kg/mm<sup>2</sup>.

4. A thermal head as set forth in claim 3; wherein the entire peripheral edge of the at least one electrode is tapered and has a taper angle of 15° or less.

5. A thermal head comprising: an insulative substrate; a heating-element layer disposed over the insulative substrate; at least one electrode disposed over the heating-element layer for supplying power to the heating-element layer, the at least one electrode having a plurality of tapered peripheral edge portions having a taper angle of 15° or less; and a protective film disposed on the at least one electrode, the protective film having a Vickers hardness of at least 1200 kg/mm<sup>2</sup>.

6. A thermal head as set forth in claim 5; wherein the at least one electrode comprises a plurality of electrodes disposed over the heating-element layer, each of the electrodes having a plurality of tapered peripheral edge portions having a taper angle of 15° or less; and wherein the protective film is disposed on the plurality of electrodes.

7. A thermal head as set forth in claim 6; wherein the tapered peripheral edge portions of each of the electrodes having a taper angle of 15° or less extend along the entire periphery of the electrodes.

8. A thermal head as claimed in claim 5; wherein the peripheral edge portions of the at least one electrode having a taper angle of 15° or less extend along the entire periphery of the at least one electrode.